

## UNITED STATES PATENT OFFICE

ALBERT C. FISCHER, OF CHICAGO, ILLINOIS, ASSIGNOR TO THE PHILIP CAREY MANUFACTURING COMPANY, A CORPORATION OF OHIO

## METHOD OF PRODUCING CONSTRUCTIONAL MATERIAL

No Drawing.

Application filed December 26, 1925. Serial No. 77,684.

This invention relates to incorporating fibrous material in bituminous material with suitable mixing contrivances and extruding the mixture in a suitable extruding machine, readily known to the art as a simplified practice of preparing fibre content premoulded expansion joints and other constructional material.

The bituminous material and fibrous matter is prepared in a suitable mechanical mixer, steam jacketed, and the mass conveyed to the chamber of the extruding machine adapted for the purpose, and the warm, fibrated mass extruded into flat premoulded strips of expansion joint. The mechanical mixers are those readily known to the art, and the extruding contrivances are those known to the art.

The purpose of my invention is to facilitate the economical production of premoulded expansion joints by bringing about a mixture of the bituminous material and fibrous material in a crisscross condition.

Usually when a mass of fibrated material is introduced between rolls, a flow is set up and the fibrous matter lays itself out in the direction of the flow, thus establishing a grain which is stronger longitudinally than it is crosswise. My invention contemplates the inter-mixture of these materials in a suitable mechanical mixer and extruding same in a suitable contrivance, thus forcing it out in a compressed state, which will not permit the fibrous material and bituminous material to set up a flow, and the fibrous material will, therefore, be incorporated in an interlaced and intertwined, crisscross condition rather than in a grain-like formation. This will produce a premoulded expansion joint which is strong in a vertical direction as well as in a horizontal direction.

Attention is particularly directed to the fact that to develop the structure as above explained it is necessary to use fibrous material of relatively long linear dimension, as dis-

tinguished from finely divided fibrous material, such as comminuted wood, or any other comminuted material which generally speaking has no definite length. When I speak of relatively long fibrous material I realize that there must necessarily be a limit as to the length of the material used, as if the fibrous material is too long considerable difficulty will be experienced in extruding the mixture. On the other hand, as heretofore explained, I am desirous of developing intertwined crisscross formation of the fibre content, and this can only be realized with fibrous material of a length to enable the same to function in this respect. There is no objection to the length of the material, so long as the extruding apparatus will accommodate. In fact I would prefer to use as long lengths as possible. Finely divided materials, such as comminuted wood, or any other comminuted material is, of course, entirely out of the question so far as developing crisscross formation of the fibre content is concerned. As an example of the material that I could use I will refer to excelsior. Of course in some instances it may be necessary to chop the excelsior into shorter lengths than that offered to the trade.

I claim:

1. The herein described method of fabricating preformed strips of elastic and resilient constructional material reenforced with linear fibers incorporated therewith in intertwined crisscross formation, which consists in mixing predetermined quantities of bituminous material and relatively long fibers, and thereafter extruding the mixture into strips of the desired dimension.

2. The herein described method of fabricating preformed strips of elastic and resilient constructional material reenforced with a fibre content incorporated therewith in intertwined crisscross formation, which consists in heating bituminous material and reducing the same to a consistency to permit of

it being thoroughly mixed with a quantity of fibers, adding fibrous material of relatively long linear dimension to the bituminous material, thoroughly mixing said materials and finally subjecting the materials to the action of an extruding apparatus to thereby extrude the material into constructional material of the desired dimension.

3. The herein described method of fabricating preformed strips of elastic and resilient constructional material reenforced with a fibre content incorporated therewith in intertwined crisscross formation, which consists in heating and thoroughly mixing bituminous material and relatively long fibers and immediately after said mixing step has been completed, extruding the mixture into constructional material of the desired dimension.

4. The herein described method of fabricating preformed strips of elastic and resilient expansion joint material reenforced with linear fibers incorporated therewith in intertwined crisscross formation, which consists in mixing predetermined quantities of bituminous material and relatively long fibers, and thereafter extruding the mixture into strips of the desired dimension.

5. The herein described method of fabricating preformed strips of elastic and resilient expansion joint material reenforced with a fiber content incorporated therewith in intertwined crisscross formation, which consists in heating bituminous material and reducing the same to a consistency to permit of it being thoroughly mixed with fibrous material, adding a quantity of fibers of relatively long linear dimension to the bituminous material, thoroughly mixing said materials and finally subjecting the materials to the action of an extruding apparatus to thereby extrude the material into strips of the desired dimension.

6. The herein described method of fabricating preformed strips of elastic and resilient expansion joint material reenforced with a fiber content incorporated therewith in intertwined crisscross formation, which consists in heating and thoroughly mixing bituminous material and relatively long fibers, and immediately after said mixing step has been completed, extruding the mixture into expansion joint material of the desired dimension.

7. The herein described method of forming preformed strips of constructional material reenforced with linear fibers incorporated therewith in intertwined crisscross formation, which consists in mixing predetermined quantities of bituminous material and relatively long fibers, and thereafter extruding the mixture into strips of the desired dimension.

8. The herein described method of forming preformed strips of constructional ma-

terial reenforced with a fiber content incorporated therewith in intertwined crisscross formation, which consists in heating and thoroughly mixing bituminous material and relatively long fibers, and immediately after said mixing step has been completed, extruding the mixture into constructional material of the desired dimension.

Signed at Chicago, Illinois, this 16th day of Dec. A. D. 1925.

ALBERT C. FISCHER.

86

80

85

90

95

100

105

110

115

120

125

130